

[54] COMPOSITE COATED STEEL STRUCTURE  
FOR CORROSION RESISTANCE

[75] Inventor: **Frederick A. Glaski**, Torrance,  
Calif.

[73] Assignee: **Fansteel Inc.**, N. Chicago, Ill.

[22] Filed: **June 4, 1973**

[21] Appl. No.: **366,284**

**Related U.S. Application Data**

[60] Division of Ser. No. 284,639, Aug. 29, 1972, Pat. No.  
3,784,403, which is a continuation-in-part of Ser. No.  
177,929, Sept. 7, 1971, Pat. No. 3,767,456.

[52] U.S. Cl. .... **29/198; 29/196; 29/196.6**

[51] Int. Cl.<sup>2</sup> .... **B23P 3/00**

[58] **Field of Search**..... 29/196, 196.6, 198;  
148/6.35, 120; 117/105.2, 107.2, 71 M

[56] **References Cited**

UNITED STATES PATENTS

|           |         |                 |                |
|-----------|---------|-----------------|----------------|
| 2,767,464 | 10/1956 | Nack et al.     | ..... 29/196   |
| 2,998,642 | 9/1961  | McCawley        | ..... 29/198   |
| 3,164,496 | 1/1965  | Hibbard et al.  | ..... 148/120  |
| 3,170,234 | 2/1965  | Tarr            | ..... 29/198   |
| 3,219,474 | 11/1965 | Priceman et al. | ..... 117/71 M |

|           |         |               |                |
|-----------|---------|---------------|----------------|
| 3,628,924 | 12/1971 | Nishio et al. | ..... 29/196   |
| 3,767,456 | 10/1973 | Glaski        | ..... 117/71 M |
| 3,784,403 | 1/1974  | Glaski        | ..... 117/71 M |

**OTHER PUBLICATIONS**

Sachs, G., et al.; Practical Metallurgy; Cleveland (ASM) 1951 p. 294, [TN 665 S 240].

Barrett, C., et al.; Structure of Metals; New York, 1966 p. 536, [TN690 B3].

*Primary Examiner*—Walter R. Satterfield

*Attorney, Agent, or Firm*—Barnes, Kisselle, Raisch & Choate

[57] **ABSTRACT**

A composite coated steel structure having a carbon steel or stainless steel base and cladding of tantalum or columbium to provide corrosion resistant surfaces for many uses. The composite includes a containment substrate coating interposed between the base and the cladding to prevent diffusion of the cladding material into the base. The containment coating has greater stability with respect to the base than the cladding material to prevent adverse reaction under high heat conditions.

**1 Claim, 1 Drawing Figure**



## COMPOSITE COATED STEEL STRUCTURE FOR CORROSION RESISTANCE

This application is a division of my copending application entitled "Process for Cladding Steel," Ser. No. 284,639, filed Aug. 29, 1972, now U.S. Pat. No. 3,784,403, issued Jan. 8, 1974 which in turn was a continuation-in-part of my copending application now entitled "Chemical Vapor Deposition of Steel with Tantalum and Columbium," Ser. No. 177,929, filed Sept. 7, 1971, and now U.S. Pat. No. 3,767,456, dated Oct. 23, 1973.

This invention relates to a Composite Coated Steel Structure for Corrosion Resistance.

There are certain applications of steel in which the product would be much enhanced by a cladding of tantalum on the surface to increase resistance to corrosion. The problem is to find an acceptable and reproducible bond between the tantalum and the steel and, secondly, to achieve uniformity over all the surfaces of a complex shape or a batch of complex-shaped hardware.

An attempt to deposit tantalum directly on steel containing carbon results in a poor bonding inasmuch as the tantalum combines with the carbon of the steel at an excessive rate leaving Kirkendall type porosity in the steel. It is possible to provide an excellent bond between tantalum and pure metals such as molybdenum, chromium and iron; but as the carbon content of the steel increases, the bond becomes less satisfactory. In steels such as the stainless variety the carbon content may be reduced to the point of not causing objectionable combining with tantalum, but the high nickel content creates the problem here. In a CVD process, the nickel will diffuse rapidly into tantalum leaving again the objectionable porosity.

The present invention contemplates a coating on steel which will protect the surface against the deterioration when tantalum is deposited by chemical vapor deposition. It is, therefore, an object of the invention to provide a process for cladding steel with tantalum or possibly columbium which is consistently successful and uniform.

It is a further object to provide a product of a tantalum clad steel resulting from the process and to provide a process which insures uniform results on complicated shapes.

Other objects and features of the invention relating to details of the process and the product will be apparent in the following description and claims in which the principles of the invention are set forth in connection with the best mode presently contemplated for the practice of the invention.

A DRAWING accompanies the disclosure and a single view thereof may be described as a diagrammatic illustration of an apparatus for accomplishing the present invention.

In connection with the problem of tantalum cladding of carbon containing steel, we propose to establish a containment surface on the steel which will prevent carbon diffusion from the steel substrate to the tantalum being deposited thereon.

By way of definition, an "overcoat" on a particular sub-strate is defined as the deposition of a measurable thickness of material on a surface. All electroplated coatings are overcoats; and, similarly, hydrogen-reduced refractory metal halides in a chemical vapor deposition process results in an overcoat. In these de-

positions, all the components of the coating are provided by the plating bath or the plating gas and none are provided by the substrate.

We propose a containment surface on a substrate which might be defined as a "displacement diffusion" coating in which at least one of the constituents of the coating is provided by the sub-strate. In this process, the coating does not build up on the surface to any appreciable extent but rather grows into the surface. For example, when titanium is used, this may be referred to as a "titanizing process." The "-izing" or "-ized" suffix placed on the end of the name of the element deposited from the gas denotes such a reaction.

In connection with titanizing, there is a reaction of the titanium with the carbon in an atmosphere of  $TiCl_4$  in the temperature range of 900°-1100°C. which forms a thin diffusion barrier of titanium carbide. The  $TiCl_4$  reacts with the surface carbon on the carbon steel substrate to form  $TiC$  and once all surface carbon is reacted, the titanium deposition ceases. Thus, there is a definite limitation on the thickness of the displacement diffusion coating. Since titanium carbide is thermodynamically more stable than  $TaC$ , the pure tantalum may be deposited without further carbon diffusion from the sub-strate. In the preparation of the displacement diffusion coating, there may be a reaction with free carbon on the surface with the  $TiCl_4$ , but, in general, the carbon is available primarily from metal carbides in the sub-strate which are less stable than  $TiC$ . Nearly all the metal carbides normally occurring in carbon steel and low alloy carbon steel are less stable than  $TaC$  and thus displacement diffusion coating is required.

While titanium has been mentioned above, it is possible to use a containment coating of a metal selected from Groups IVb and VIb, iron, and cobalt, of this group, for example, titanium carbide and  $ZrC$  are both more stable than tantalum carbide. After this containment coating is applied, it is possible to overcoat with pure tantalum in a CVD process without further carbon diffusion from the sub-strate.

In connection with stainless steels which are high in chromium and nickel, the problem with carbon diffusion is reduced since the carbide with chromium, namely,  $Cr_7C_3$ , is very stable. On the other hand, the nickel content of the stainless steel will diffuse uncontrollably into a tantalum clad coat. Thus, for these steels, an overcoat of the pure metal to which tantalum may be bonded in a CVD process must be used. In some instances, a plating process may be used and in other instances a plasma spray can provide a coating to which tantalum may successfully bond. In each case, care must be used to obtain a good bond between the sub-strate and the overcoat. With electroplating, careful pre-plating procedures must be observed in the cleaning of the part and well controlled plating steps must be utilized. In the plasma spraying, a coating of pure iron, chromium, cobalt, molybdenum or tungsten may be applied; in fact, any of the metals from Group IVb and Group VIb as well as iron or cobalt can be practically applied in this way.

Once the pure metal overcoat is applied to the stainless steel, the nickel diffusion is blocked and the CVD coating or clad of tantalum can be readily applied using conventional procedures.

It will be appreciated that carbon steel can also be plated or plasma sprayed with pure metals as above de-

scribed to block carbon diffusion. With steel castings, for example, they are sometimes ground out and plasma coated with iron to remove the surface porosity and then titanized to stabilize any carbon that may have diffused into the plasma coat. Then the tantalum clad may proceed with a resulting good quality and uniform coat.

With respect to the use of plasma spray of iron or stainless steel, the carbon diffusion is not as critical a problem since the iron interlayer remains pure iron and the bonding of the CVD tantalum readily occurs without titanizing.

It has also been noted in tantalum cladding that deposition has occurred preferentially on certain areas of exposed parts rather than uniformly or in the areas where it is most generally desired. Tantalum cladding has been much improved by a control of the mixing of the tantalum  $\text{Cl}_5$  and the hydrogen reactant gases.

In the chemical vapor deposition process which otherwise proceeds in accordance with accepted procedures in a reduction reaction, better results have been obtained when the  $\text{TaCl}_5$  is introduced to the chamber in the normal manner as indicated in the drawing. However, the hydrogen is introduced through a separate feed line or a plurality of feed lines which terminate immediately upstream of the object to be coated. In other words, the gases are intentionally separated until they impinge on the object to be coated. This provides excellent control in putting the tantalum deposit where it is desired. Utilizing this technique, uniform tantalum claddings have been obtained on batches of cast valve bodies, for example, during a 45-minute deposition period in a system that formerly could not generate tantalum coverage over all areas of the valve bodies during a 5-hour period of deposition. Thus, there is a great savings in materials and expense in performing the process as well as a much more desirable and uniform result. In some instances, a control of this combined flow which is brought together immediately upstream of the area to be plated can be improved by using multiple exhaust ports which are balanced to direct the flow to certain areas of the parts to be exposed.

While the above description has referred to tantalum cladding, it will be appreciated that columbium (niobium) is chemically similar and may be applied as a cladding coat in the same way as has been described in connection with tantalum. The same problems which require a containment coat for tantalum exist in relation to columbium. There is a considerable savings in the use of columbium since it is a less expensive metal but, on the other hand, tantalum has a broader applicability as a corrosion resistant material.

The term "coating" or "coat" as used in the specification and claims has reference to the application, by CVD, plating, or plasma spray, to a sub-strate surface of a metal in an extremely thin layer under conditions as above described in which the metal unites with the surface carbon of the sub-strate to form a carbide having greater stability than tantalum carbide. The surface is thus prepared for the application of tantalum by chemical vapor deposition to the extent that there will be no perceptible formation of tantalum carbide at the bonding face. The above description of coating relates to metals from Group IVb and the coating may also include metals from Group VIb, iron and cobalt applied as a pure metal to reduce the carbon diffusion during the tantalum coating.

Following are three examples of a process used for steel cladding with sub-strates of differing carbon and stainless steels and various treatments prior to the titanizing and the application of the tantalum clad.

#### EXAMPLE 1

Cladding of 6 inches I.D.  $\times$  24 inches long pipe spool made of type A-106 Carbon Steel

1. Sand blast surface to remove scale and roughen surface for subsequent plasma sprayed coating.
2. Plasma spray 0.002 inch thick coating of iron on I.D. and flange seal faces.
3. Place in CVD (chemical vapor deposition) furnace, evacuate with vacuum pump and heat to titanizing temperature of 1,070°C. in argon.
4. Bubble hydrogen at 2 liters/minute through liquid  $\text{TiCl}_4$  and mix with the resultant gas 7 liters/minute of pure hydrogen (STP) and flow the mixture through spool, over flange seal faces and I.D. surface for one-half hour at 1,070°C. and -23 inches Hg. pressure.
5. After titanizing, adjust temperature to 1,010° - 1,040°C. range and begin tantalum deposition by flowing 3 liters/minute of chlorine through heated tantalum chips to form  $\text{TaCl}_5$  and mixing the resultant gas with 18 liters/minute of hydrogen, passing it through the spool at 34 torr pressure. All gas flows at STP.
6. After one-half hour, adjust gas flows to 7.5 liters/minute of chlorine and 45 liters/minute of hydrogen, both at STP.
7. Total tantalum deposition time 6  $\frac{1}{2}$  hours.
8. Turn off chlorine and hydrogen and cool in argon.
9. Resultant deposit thickness from 0.009 to 0.015 inch over both flange seal faces and I.D. of spool.

#### EXAMPLE 2

Cladding of type 316SS pump housing with 1 inch ports and flanges and 4  $\frac{1}{2}$  inches diameter cavity

1. Degrease and descale in HCl - base commercial descaler solution.
2. Place in CVD furnace, evacuate with vacuum pump and heat to titanizing temperature at 1,000°C. in argon.
3. Bubble hydrogen at 2 liters/minute (STP) through liquid  $\text{TiCl}_4$  and mix the resultant gas with 7 liters/minute of pure hydrogen and flow the mixture through pump housing, over flange seal faces and inside surface for 1 hour at 1,000°C. and -23 inches Hg. pressure.
4. After titanizing, adjust temperature to 1,010° - 1,030°C. range and begin tantalum deposition by flowing 1.5 liters/minute of chlorine through heated tantalum chips to form  $\text{TaCl}_5$  and mixing with 9 liters/minute of hydrogen, passing the mixture through the pump housing at 30 torr pressure. All gas flows at STP.
5. Total tantalum deposition time 5  $\frac{1}{2}$  hours.
6. Turn off chlorine and hydrogen and cool in argon.
7. Resultant deposit thickness from 0.012 inch to 0.020 inch over both flange faces and inside surface of pump housing.

#### EXAMPLE 3

Cladding of type 1215 carbon steel thermowell, three-fourths inch diameter  $\times$  4 inches long well with 2  $\frac{1}{2}$  inches diameter (flat-to-flat)  $\times$  2 inches long hexagonal base. Total length 6 inches

1. Degrease and descale in HCl - base commercial descaler solution.

2. Place in CVD chamber, evacuate with vacuum pump to heat directly by induction to titanizing temperature at 1,100° – 1,125°C. after baking in H<sub>2</sub> at 1,050° – 1,075°C. for 10 minutes.

3. Bubble H<sub>2</sub> at 800 cc/minute through liquid TiCl<sub>4</sub> and mix the resultant gas with 3.5 liters/minute of pure hydrogen (STP) and flow the mixture over the outer surface of thermowell for 15 minutes at 1,100° – 1,125°C. and –15 inches Hg. pressure.

4. After titanizing, adjust temperature to tantalum deposition range, 1,010° – 1,030°C. and flow Cl<sub>2</sub> at 1 liter/minute through heated tantalum chips to form TaCl<sub>5</sub> and mix the resultant gas with 6.25 liters/minute of hydrogen passing the mixture over the thermowell surface at 30 torr pressure. All gas flows at STP. 10

5. Total tantalum deposition time 75 minutes.

6. Turn off chlorine and hydrogen and cool in argon.

7. Deposit thickness from 0.007 inch at underside of hexagon adjacent to threaded coupling, to 0.010 inch – 1.020 inch on remaining well surface (0.020 inch at 20 the tip).

It will be noted that the example using stainless steel shows a longer exposure time and a lower temperature

than the examples on carbon steel. This is required to avoid eutectic melting by the titanium and nickel in the steel. This melting would occur at "normal" carbon steel titanizing temperatures.

I claim:

1. A composite structure having a corrosion resistant surface which comprises:

a. a non-refractory steel substrate containing free carbon and metal carbides,

b. a displacement diffusion containment coating on said substrate to isolate carbon and metal carbides from the surface of the substrate composed of titanium carbide formed from an in situ combination of titanium with the carbon and metal carbides of the substrate, said displacement diffusion coating being stable in the presence of tantalum or columbium at temperatures ranging from 900° to 1,100°C., and

c. a corrosion resistant material selected from the group consisting of tantalum and columbium molecularly bonded to said containment coating by chemical vapor deposition.

\* \* \* \* \*

25

30

35

40

45

50

55

60

65